# EUROPEAN PATENT SPECIFICATION

(11) **EP 2 910 309 B1**
(45) Date of publication and mention of the grant of the patent: **27.07.2022**
(21) Application number: 13846992.9
(22) Date of filing: 11.10.2013
(51) Int. Cl.: B03C 1/033, B03C 1/18

(54) **MAGNETIC SORTING APPARATUS, MAGNETIC SORTING METHOD, AND METHOD FOR MANUFACTURING IRON SOURCE**
MAGNETISCHE SORTIERVORRICHTUNG, MAGNETISCHES SORTIERVERFAHREN UND VERFAHREN ZUR HERSTELLUNG EINER EISENQUELLE
APPAREIL DE TRI MAGNÉTIQUE, PROCÉDÉ DE TRI MAGNÉTIQUE ET PROCÉDÉ DE FABRICATION DE SOURCE DE FER

(30) Priority: 16.10.2012 JP 2012229214; 16.10.2012 JP 2012229210
(43) Date of publication of application: 26.08.2015
(73) Proprietor: JFE Steel Corporation, Tokyo, 100-0011 (JP)
(72) Inventor: ISHIDA, Kyohei, Tokyo 100-0011 (JP); NISHINA, Yoshiaki, Tokyo 100-0011 (JP); ENOEDA, Seiji, Tokyo 100-0011 (JP); IMANISHI, Daisuke, Tokyo 100-0011 (JP)
(74) Representative: Grünecker Patent- und Rechtsanwälte PartG mbB
(86) International application number: PCT/JP2013/006109
(87) International publication number: WO 2014/061256

(56) References cited:
- CN-U- 202 087 414
- CN-Y- 200 981 018
- DE-A1- 19 838 170
- JP-A- 2008 104 915
- JP-A- 2011 104 583

## Description

### [Technical Field]

The present invention relates to a technology to magnetically separate (separate) ferromagnetic particles from a powder and granular material containing the ferromagnetic particles and relates to, for example, a magnetic separator and a magnetic separation method, which are suitable for separating an iron content from a slag obtained as a by-product of an ironmaking process, and a method for manufacturing an iron source.

### [Background Art]

In the ironmaking process, a slag (steelmaking slag) is generated as a by-product in a molten pig iron pretreatment or a converter decarbonization step. The slag is generated on the basis of reaction of a calcium based additive added to remove impurities and unnecessary elements in the molten pig iron and a molten steel (sometimes iron and steel are collectively called iron) with these impurities and unnecessary elements. Besides the removed impurities and unnecessary elements, a high proportion of iron content is also contained in the slag.

In order to recycle the iron content in the slag, the iron content has been separated and recovered. Usually, the iron content is separated and recovered by the following steps. Initially, the slag is sieved to remove large (several hundreds of millimeters) blocks included in the slag. In small blocks passed through a sieve, an iron content and a slag content adhere to each other. Therefore, rough crushing into the size of several tens of micrometers to several tens of millimeters is performed with a hammer crusher, a rod mill, or the like to facilitate liberation (separation of the iron content from the slag content). Thereafter, the iron content is separated with a magnetic separator. In general, examples of apparatuses used as the magnetic separator include suspended electro magnets, magnetic drum separators, and magnetic pulleys.

Also, in order to liberate an iron content, in some cases, a slag is heated and is cooled for an appropriate time, followed by crushing. It is possible to separate only the adhering slag content without crushing iron blocks or micronize the slag into several tens of micrometers depending on the cooling time.

It is needless to say that liberation proceeds as micronization of the slag proceeds regardless of the method.

In general, in order to increase the recovery rate of the iron content, it is necessary to pursue liberation. Therefore, the particle diameter of the slag is reduced by repeating mechanical crushing. Alternatively, the diameter may be reduced by a heat treatment.

In the case where magnetic separation is performed to recover the iron content, for example, a magnetic separator shown in Fig. 8 has been previously used (for example, NPL 1). This apparatus is a magnetic pulley type (belt conveyer style) magnetic separator, where a powder and granular material (a) containing ferromagnetic particles is supplied from a supply device 23 onto a conveyer belt 20, and ferromagnetic particles and non-magnetic particles are separated when the powder and granular material a is discharged from a conveyer end edge portion 27. In the inside of a belt guide roll 21 on the conveyer end edge portion 27 side, magnets 22 are disposed in part of the circumferential direction. The magnets 22 are disposed in such a way that magnetic poles adjacent in the circumferential direction of the belt guide roll 21 are different from each other. The magnets 22 are stationary magnets disposed independently of the belt guide roll 21.

In this magnetic separator, the magnetic forces of the magnets 22 inside the belt guide roll 21 act on the powder and granular material a on the conveyer belt 20 in the conveyer end edge portion 27, non-magnetic particles not attracted by the magnets 22 fall first so as to be recovered by a magnetically not-attracted material recovery portion 24y, and the ferromagnetic particles attracted by the magnets 22 pass through a partition plate 25 disposed below the belt guide roll 21 and fall at positions at which the magnetic force is weakened, so as to be recovered by a magnetically attracted material recovery portion 24x.

The document DE19838170 A1 is concerned with a belt-type magnetic separator in which a particle stream is separated by a magnetic field over a conveyor. This induces force and moment in conductive particles; depending on their nature, they are levitated and then fall to the ground through different trajectories. The magnetic wheel of the separator has a conveyor belt running around it, which assists separation and interception of ferromagnetic particles. Particles affected by the field are fractionated in accordance with the lengths of their trajectories, which stem from their properties.

### [Citation List]

### [Patent Literature]

[PTL 1] Japanese Unexamined Patent Application Publication No. 2006-142136
[PTL 2] Japanese Unexamined Patent Application Publication No. 10-130041

### [Non Patent Literature]

[NPL 1] J. Svoboda, Magnetic Techniques for the Treatment of Materials, pp. 70-72, Kluwer Academic Publishers, 2004

### [Summary of Invention]

### [Technical Problem]

However, as shown in Fig. 8, in the case where a large amount of powder and granular material a is supplied to a previously known magnetic separator and the layer thickness of the powder and granular material a increases, the following problem occurs. The micronized powder and granular material a is in the state in which ferromagnetic particles enclose non-magnetic particles, and the ferromagnetic particles and the non-magnetic particles are attracted by the magnet 22 at the same time, so that the ferromagnetic particles and the non-magnetic particles are not separated from each other easily. This becomes considerable as the particle diameter of the powder and granular material a decreases. Furthermore, an agglomeration phenomenon due to micronization is added, so that in the case where the layer thickness of the powder and granular material a on the conveyer belt 20 increases, as shown in Fig. 8, non-magnetic particles are also allowed to enter the magnetically attracted material recovery portion 24x, and the ferromagnetic particles cannot be separated appropriately.

It is necessary to deal with the above-described problem usually in such a way that, for example, as shown in Fig. 9, the amount of supply of powder and granular material a is decreased by utilizing a vibrating feeder 26 or the like to reduce the thickness of the powder and granular material layer on the conveyer belt 20 to, such as, the thickness of about one or two particles. However, if the amount of supply of the powder and granular material a is decreased, the treatment speed is reduced, although the performance to separate the ferromagnetic particles is ensured. In the case of magnetic separation of a slag, several tons to several tens of tons per hour of treatment is necessary and, therefore, it is indispensable to perform a large amount of magnetic separation in a short time. Consequently, it is difficult for the above-described previously known magnetic separator to magnetically separate a large amount of powder and granular material a in a short time.

On the other hand, PTL 1 proposes a method in which foreign matters are separated without over-crushing the slag by undergoing a plurality of specific steps. However, there is a problem that the separation flow becomes complicated and the treatment cost increases. Also, as shown in PTL 2, a wet process is commonly applied in order to avoid agglomeration, but there is a problem that a waste fluid disposal cost increases considerably.

It is an object of the present invention to solve the above-described issues in the related conventional art and provide a magnetic separator and a magnetic separation method, where ferromagnetic particles are separated from a powder and granular material efficiently and magnetic separation can be performed at a low cost without the need for complicated steps and waste fluid disposal even in the case where a large amount of powder and granular material containing ferromagnetic particles is treated and in the case where the layer of a supplied powder and granular material is thick.

### [Solution to Problem]

The present inventors obtained the following findings on the magnetic separation.

In the case where ferromagnetic particles are separated from a powder and granular material, in which ferromagnetic particles and non-magnetic particles are mixed, through the use of moving magnets, when the movement of each particle is observed, initially, the ferromagnetic particle is moved in such a way as to be attracted by the magnet. The attractive force that acts on the ferromagnetic particle is changed on the basis of the change in the strength of the magnetic field in association with the movement of the magnet. When the magnetic field is strong, the ferromagnetic particles are gathered together on the basis of the attractive force. Conversely, when the magnetic field is weak, there is a tendency to disperse.

This change in the attractive force exerts an effect like vibration on the powder and granular material. The state of sandwiching and enclosure of non-magnetic particles by ferromagnetic particles is resolved on the basis of repetition of the change in the strength of the magnetic field. As a result, separation of the ferromagnetic particles from the non-magnetic particles is facilitated. Furthermore, the torque is added to the ferromagnetic particles on the basis of changes in the direction of the magnetic field, so that the ferromagnetic particles are moved between the non-magnetic particles toward the magnet side while being rotated. Most of the ferromagnetic particles are gathered gradually in the vicinity of the magnet by these two effects, and the non-magnetic particles are moved to the side farther from the magnet conversely. In this manner, the ferromagnetic particles can be separated from the non-magnetic particles by utilizing the changes in the strength and the direction of the magnetic field.

Fig. 1 (A) to (D) schematically show the above-described actions. In Fig. 1 (A) to (D), the magnetic poles of the magnet of the portion facing the powder and granular material are referred to as the north pole and the south pole. When the magnet is moved from the state in which the ferromagnetic particles on the conveyer belt 2 are attracted by the north pole, as shown in Fig. 1 (A), to the state in which a space portion between the north pole and the south pole faces the powder and granular material, as shown in Fig. 1 (B), the magnitude of the attractive force acted on the ferromagnetic particles is changed because of the strength of the magnetic field. Also, the ferromagnetic particles are attracted in the direction of arrows because of the change in the magnetic pole from the north pole to the south pole and are moved to the magnet side while being rolled. Thereafter, as shown in Fig. 1 (C), the ferromagnetic particles are attracted by the south pole and are further moved to the magnet side. The above-described actions are repeated and, thereby, the ferromagnetic particles originally distributed in the whole powder and granular material layer are gathered to the side nearest to the magnet in the powder and granular material layer, as shown in Fig. 1 (D).

This phenomenon always occurs if at least one of the magnet and the powder and granular material a is moved, and the same goes for the case where the magnet is fixed and only the powder and granular material a is moved.

In the case where the magnets are moved while the same magnetic poles are arranged side by side, movement of the ferromagnetic particles due to the changes in the strength of the magnetic field occur but the amounts of movement of the ferromagnetic particles are reduced because the torque due to the changes in the direction of the magnetic field is not added to the ferromagnetic particles. As a result, the separation efficiency is reduced.

In this regard, Fig. 1 (A) to (D) show the case where the magnets are moved from the right side to the left side in the drawing, although the same goes for the case where the magnets are moved from the left side to the right side in the drawing, in theory.

The present inventors found that the ferromagnetic particles were able to be magnetically separated efficiently by applying the above-described mechanism to a belt conveyer style magnetic separator, disposing magnets inside the belt guide roll on the conveyer end edge side in such a way that adjacent magnetic poles in the portion facing the powder and granular material were arranged to become different from each other along the circumferential direction of the belt guide roll and, in addition, in such a way that adjacent magnetic poles in the portion facing the powder and granular material were arranged to become the same in the width direction of the belt guide roll, and moving the powder and granular material in the magnetic field formed by these magnets. The effect is further enhanced by rotating the magnets and, thereby, changing the strength and the direction of the magnetic field acted on the ferromagnetic particles at a high speed.

The present invention has been made on the basis of the above-described findings and it is defined by a magnetic separator in accordance with claim 1, a magnetic separation method in accordance with claim 5 and a method for manufacturing an iron source in accordance with claim 7. Further embodiments are defined in the dependent claims.

### [Advantageous Effects of Invention]

According to the present invention, ferromagnetic particles are separated from a powder and granular material containing the ferromagnetic particles in one separation step efficiently and magnetic separation can be performed at a low cost without the need for complicated steps, waste fluid disposal, and the like even in the case where a large amount of powder and granular material containing ferromagnetic particles is treated and in the case where the layer of a supplied powder and granular material is thick.

### [Brief Description of Drawings]

[Fig. 1] Fig. 1 (A) to (D) are explanatory diagrams schematically showing actions of a magnetic separator according to the present invention.
[Fig. 2] Fig. 2 is an explanatory diagram showing a magnetic separator according to a first embodiment of the present invention and an embodiment of a magnetic separation method by using this apparatus.
[Fig. 3] Fig. 3 is a perspective view showing the structure of a belt guide roll of the magnetic separator according to the first embodiment shown in Fig. 2.
[Fig. 4] Fig. 4 is an explanatory diagram showing a modified example 1 of the magnetic separator according to the first embodiment of the present invention and a magnetic separation method by using this apparatus.
[Fig. 5] Fig. 5 is an explanatory diagram showing a modified example 2 of the magnetic separator according to the first embodiment of the present invention and a magnetic separation method by using this apparatus.
[Fig. 6] Fig. 6 is a perspective view showing the structure of a belt guide roll of a modified example 3 of the magnetic separator according to the first embodiment shown in Fig. 2.
[Fig. 7] Fig. 7 is an explanatory diagram showing a magnetic separator not covered by the claimed invention and an example of a magnetic separation method by using this apparatus.
[Fig. 8] Fig. 8 is an explanatory diagram showing a magnetic separator in the related conventional art and a state of use in the case where a large amount of powder and granular material is treated by using this apparatus.
[Fig. 9] Fig. 9 is an explanatory diagram showing a magnetic separator in the related conventional art and a state of use in the case where a small amount of powder and granular material is treated by using this apparatus.

### [Description of Embodiments]

A magnetic separator and a magnetic separation method according to the present invention are to separate ferromagnetic particles from a powder and granular material containing the ferromagnetic particles by a magnetic force. The magnetic separator according to the present invention includes a belt to carry the powder and granular material, a rotatable belt guide roll having an outer circumference partly wound with the above-described or an other belt, and a magnetic field application device provided with a plurality of magnets disposed inside the guide roll. The magnets are arranged in such a way that the magnetic poles of the portion facing the powder and granular material come into alternate sequence along the circumferential direction of the belt guide roll and, in addition, are arranged in such a way that the magnetic poles of the portion facing the powder and granular material become the same in the width direction of the belt guide roll. In the case where the magnetic poles are the same in the width direction, a uniform magnetic field is formed and the force acted on the ferromagnetic particles also becomes uniform, and the separation efficiency of the ferromagnetic particles can be enhanced.

The magnetic separation method according to the present invention separates ferromagnetic particles from a powder and granular material containing the ferromagnetic particles by using the magnetic separator having the above-described configuration.

In the magnetic separator and the magnetic separation method according to the present invention, the magnetic field change frequency F (Hz), which is defined by the following formula (1) and which indicates changes in the strength of the magnetic field acted on the powder and granular material from the magnetic field application device, is specified to be 170 Hz or more. The magnetic field change frequency F is more preferably 200 Hz or more. $F = \left(x⋅P\right) / 60$ where x: the number of revolutions per minute of magnet roll (rpm)
P: the number of magnetic poles provided to magnet roll and disposed in the circumferential direction of magnet roll (in this regard, as for the number of magnetic poles, a pair of the north pole and the south pole adjacent in the circumferential direction of the surface facing the powder and granular material (a) of the magnet roll 4r is counted as one magnetic pole and, for example, in the case where the north pole [a], the south pole [b], and the north pole [c] are aligned in the circumferential direction, the pair of the north pole [a] and the south pole [b] is counted as one magnetic pole and the pair of the south pole [b] and the north pole [c] is counted as one magnetic pole)

High-speed changes in the strength and the direction of the magnetic field acted on the powder and granular material are allowed to occur by specifying the magnetic field change frequency F (Hz) of the magnetic field application device to be 170 Hz or more, and preferably 200 Hz or more, so that it becomes possible to separate the ferromagnetic particles contained in the powder and granular material accurately.

### [First embodiment]

Fig. 2 is an explanatory diagram showing a magnetic separator according to a first embodiment of the present invention and an embodiment of a magnetic separation method by using this apparatus.

The apparatus according to the first embodiment includes a first belt conveyer A to carry a powder and granular material (a) and a second belt conveyer B which is located above the belt conveyer A and which attracts and separates ferromagnetic particles, by magnets, from the powder and granular material a carried with the belt conveyer A.

In the first belt conveyer A, reference numeral 1 denotes a conveyer belt, reference numeral 8 denotes a belt guide roll on the conveyer start edge portion 14 side, and reference numeral 9 denotes a belt guide roll on the conveyer end edge portion 10 side. The conveyer belt 1 is disposed between the belt guide rolls 8 and 9 and, thereby, the belt conveyer A is constructed.

In the second belt conveyer B, reference numeral 2 denotes a conveyer belt, reference numeral 3 denotes a belt guide roll at the conveyer start edge portion 11 side, and reference numeral 13 denotes a belt guide roll at the conveyer end edge portion 12 side. The conveyer belt 2 is disposed between the belt guide rolls 3 and 13 and, thereby, the belt conveyer B is constructed. In the present first embodiment, the belt guide roll 3 is configured to have a diameter larger than the diameter of the belt guide roll 13 and the axis of rotation of the belt guide roll 13 is located upper than the axis of rotation of the belt guide roll 3, so that the upper surface of the conveyer belt 2 (an upper belt portion between the belt guide rolls 3 and 13) is almost horizontal. However, the upper surface of the conveyer belt 2 may come down toward the belt guide roll 13.

A supply device 6 to supply the powder and granular material a containing the ferromagnetic particles is disposed above the conveyer belt 1 and at the position near to the conveyer start edge portion 14 of the belt conveyer A.

The ferromagnetic particles attracted and held on the belt conveyer B side are carried with the belt conveyer B and, thereafter, discharged from the conveyer end edge portion 12. Therefore, a magnetically attracted material recovery portion 7x is disposed below the conveyer end edge portion 12 of the belt conveyer B. Also, non-magnetic particles fall below the conveyer start edge portion 11 of the belt conveyer B, so that a magnetically not-attracted material recovery portion 7y is disposed at that position.

In the first embodiment shown in Fig. 2, the conveyer start edge portion 11 of the belt conveyer B is closely located above the conveyer end edge portion 10 of the belt conveyer A. In this regard, the belt guide rolls 8 and 9 of the belt conveyer A and the belt guide rolls 3 and 13 of the belt conveyer B are rotated in the directions reverse to each other and the conveyer belts 1 and 2 are moved in the same direction in the conveyer end edge portion 10 of the belt conveyer A and the conveyer start edge portion 11 of the belt conveyer B.

In the belt conveyer B, any one of the belt guide rolls 3 and 13 may be a driven roll driven by a drive device, e.g., a motor. However, usually, the belt guide roll 13 is a driven roll and the belt guide roll 3 is a non-driven roll. The belt guide roll 3 is formed from a sleeve body with a hollow inside and is rotatably supported.

In the first embodiment, a magnet roll 4r serving as a magnetic field application device provided with a plurality of magnets 5 is disposed inside the belt guide roll 3. The magnet roll 4r is configured to be be able to rotate independently of the belt guide roll 3.

As shown in Fig. 3 described later, in the first embodiment, the magnet roll 4r is provided with the plurality of magnets 5 at predetermined intervals in the circumferential direction and the width direction of the belt guide roll 3. The plurality of magnets 5 are arranged with magnetic poles aligned in such a way that alternating north poles and south poles adjoin over 360° in the roll circumference direction of the magnet roll 4r. Also, the plurality of magnets 5 are arranged in such a way that the same magnetic poles are aligned in the width direction of the magnet roll 4r.

The number of magnets 5 arranged in the roll circumferential direction, the interval of the magnets 5, and the like are not specifically limited. Higher speed of changes in the strength and the direction of the magnetic field are obtained by increasing the number of the magnets 5 or reducing the interval of the magnets 5. Put another way, high-speed changes in the magnetic field are obtained even when the rotational speed of the magnet roll 4r is low.

The strength of the magnetic field due to the magnets 5 is not specifically limited. Usually, the magnets 5 are selected in such a way that about 0.01 to 0.5 T is ensured in the conveyer belt portion in contact with the belt guide roll 3 in accordance with an object. If the magnetic field is too weak, the effect of the magnet roll 4r is not obtained sufficiently. On the other hand, if the magnetic field is too strong, the attractive force acted on the ferromagnetic particles is too strong and, on the contrary, separation of the ferromagnetic particles may be hindered.

Meanwhile, in the apparatus according to the first embodiment, the magnetic field is switched in the manner of strong → weak → strong → weak → ··· and the effect on the ferromagnetic particles in the powder and granular material layer is repeated in the manner of gathering → dispersion → gathering → dispersion → ··· because of the plurality of magnets 5 arranged at the predetermined interval and the space portions between adjacent magnets 5. The width of space portions between magnets 5 adjacent in the circumferential direction is not specifically limited, although about 1 to 50 mm is appropriate to obtain the above-described effects.

Fig. 3 is a perspective view showing the structure of the belt guide roll of the magnetic separator according to the first embodiment shown in Fig. 2. The magnet roll 4r provided with the plurality of magnets is disposed inside the belt guide roll 3. Reference numeral 40 denotes a roll shaft of the magnet roll 4r. Roll shafts 30 at both ends of the belt guide roll 3 are allowed to cover the roll shaft 40 of the magnet roll 4r disposed inside the belt guide roll 3 and are fitted to the roll shaft 40 with a bearing 15 (metal bearing, roller bearing, or the like) therebetween.

However, the belt guide roll 3 and the magnet roll 4r can be rotated independently of each other and the roll shaft 30 and the roll shaft 40 can take various forms.

The magnet roll 4r is a roll rotated by a device, e.g., a motor, and the rotational direction thereof may be the same as or reverse to the direction of the belt guide roll 3. In general, the rotation is in the direction reverse to the direction of the belt guide roll 3. In this regard, the magnet roll 4r is rotated at a speed higher than the speed of the belt guide roll 3.

In the present first embodiment, it is preferable that changes in the magnetic field occur at a maximized speed (high-speed changes in the strength and the direction of the magnetic field). Specifically, as described above, the magnetic field change frequency F (Hz), which is defined by the following formula (1), of the magnet roll 4r is specified to be preferably 170 Hz or more. The magnetic field change frequency is more preferably 200 Hz or more.$F = \left(x⋅P\right) / 60$ where x: the number of revolutions per minute of magnet roll 4r (rpm)
P: the number of magnetic poles provided to magnet roll 4r (in this regard, as for the number of magnetic poles, a pair of the north pole and the south pole adjacent in the circumferential direction of the surface facing the powder and granular material (a) of the magnet roll 4r is counted as one magnetic pole) and, for example, in the case where the north pole [a], the south pole [b], and the north pole [c] are aligned in the circumferential direction, the pair of the north pole [a] and the south pole [b] is counted as one magnetic pole and the pair of the south pole [b] and the north pole [c] is counted as one magnetic pole. For example, in the case where 12 poles (a pair of the north pole and the south pole is counted as one magnetic pole) of magnets (for example, neodymium magnets) are disposed in the circumferential direction, when the rotational speed of the magnet roll 4r is specified to be 1,000 rpm, the magnetic field change frequency results in 200 Hz. Also, in the case where 24 poles (a pair of the north pole and the south pole is counted as one magnetic pole) of magnets are disposed in the circumferential direction and the magnetic field change frequency is specified to be 200 Hz likewise, the rotational speed of the magnet roll 4r may be 500 rpm.

The upper limit of the magnetic field change frequency is about 1,000 Hz because there is a mechanical upper limit to the number of revolutions per minute of the magnet roll 4r and the effect of changes in the magnetic field may be saturated even when the frequency is increased.

The size of the magnet 5 is not specifically limited insofar as the size is suitable for arranging the predetermined number of magnets 5. In this regard, in Fig. 2, the magnetic poles of one magnet 5 are arranged in such a way that the magnetic pole on the inner circumferential side of the magnet roll 4r is different from the magnetic pole on the outer circumferential side. However, as a matter of course, the magnets 5 may be disposed in such a way that the different magnetic poles of one magnet 5 are arranged in the circumferential direction of the magnet roll 4r. In this case as well, the north pole and the south pole are disposed alternately, so that the ferromagnetic particles can be separated efficiently. The north pole and the south pole may be disposed with a space portion therebetween. Alternatively, the north poles may be disposed with a space portion therebetween and the south poles may be disposed with a space portion therebetween.

In addition, the space portions between the magnets 5 may be filled with a resin or the like, and a cover may be attached to the outer circumference of the magnet roll 4r.

The rotational direction of the magnet roll 4r may be either (i) the direction reverse to the movement direction of the conveyer belt 2 (the rotational direction of the belt guide roll 3) or (ii) the same direction as the movement direction of the conveyer belt 2 (the rotational direction of the belt guide roll 3). A carrying force is exerted on the ferromagnetic particles to move in the direction reverse to the rotational direction of the magnet roll 4r because of the action of the magnetic field of the rotating magnet roll 4r. In the case of the above-described item (i), the carrying force exerted on the ferromagnetic particles by the magnetic field and the frictional force between the conveyer belt 2 and the ferromagnetic particles become the same direction. On the other hand, in the case of the above-described item (ii), the directions of the above-described carrying force and frictional force become reverse to each other. However, the frictional force is larger in this case and, therefore, the ferromagnetic particles are carried in the movement direction of the conveyer belt 2.

When the item (i) and the item (ii) are compared, in the case of the item (ii), the directions of the carrying force exerted on the ferromagnetic particles by the magnetic field and the frictional force between the conveyer belt 2 and the ferromagnetic particles become reverse to each other, so that the ferromagnetic particles may stay on the conveyer belt 2, although the ferromagnetic particles can be separated more efficiently. On the other hand, in the case of the item (i), the ferromagnetic particle separation efficiency is slightly lower than that in the case of the item (ii), but the ferromagnetic particles do not stay on the conveyer belt 2 and, therefore, there is an advantage that the particles can be carried smoothly.

The function and the operation of the magnetic separator according to the present first embodiment and the magnetic separation method by using this apparatus will be described below.

In the magnetic separator according to the present first embodiment, the belt feed speeds of the conveyer belts 1 and 2 of the belt conveyers A and B may be specified to be speeds required for the treatment process. Then, in the case of the magnetic separator shown in Fig. 2, the rotational speed of the magnet roll 4r is determined in such a way that the speed of changes in the magnetic field becomes sufficiently high relative to this belt feed speed. In particular, it is preferable that the rotational speed of the magnet roll 4r be set in such a way as to satisfy the above-described condition represented by the formula (1).

A sufficient thickness of powder and granular material a containing the ferromagnetic particles is supplied from the supply device 6 to the moving conveyer belt 1 of the belt conveyer A, while the belt conveyers A and B are operated. This powder and granular material a is carried to the conveyer end edge portion 10. The upper surface of the powder and granular material a carried with the conveyer belt 1 is brought into contact with the lower surface of the conveyer start edge portion 11 of the belt conveyer B in the vicinity of the conveyer end edge portion 10, and the powder and granular material a slips between the conveyer end edge portion 10 of the belt conveyer A and the conveyer start edge portion 11 of the belt conveyer B. At this time, the magnetic field of the magnetic field application device 4 of the belt conveyer B is exerted on the powder and granular material a.

In this regard, in the case of the magnetic separator shown in Fig. 2, the ferromagnetic particles in the form of enclosing non-magnetic particles in the powder and granular material a are attached to the lower surface side of the belt conveyer B because of the magnetic force of the magnet roll 4r serving as the magnetic field application device 4 and are carried with the conveyer belt 2. The ferromagnetic particles in the powder and granular material a undergo action of the magnetic field of the magnets 5 included in the magnet roll 4r and the strength of the magnetic field is switched in the manner of strong → weak → strong → weak → ··· instantaneously because of the rotation of the magnet roll 4r. The effect in the manner of gathering → dispersion → gathering → dispersion → ··· is repeated on the ferromagnetic particles in the powder and granular material layer.

Also, in the case where the magnetic field application device is formed from the magnet roll 4r which is rotated independently of the belt guide roll 3, as in the embodiment shown in Fig. 2, the ferromagnetic particles can be efficiently magnetically separated even when the thickness of the powder and granular material a supplied to the conveyer belt 1 is sufficiently increased, as shown in Fig. 2, because of the functions of (1) mechanically generating high-speed changes in the magnetic field by rotating the magnet roll 4r, (2) supplying the powder and granular material a with a sufficient layer thickness into the resulting changing magnetic field, (3) moving the ferromagnetic particles to the magnet roll 4r side and excluding the non-magnetic particles to the side apart from the magnet roll 4r while entanglement and enclosure of the non-magnetic particles by the ferromagnetic particles are resolved on the basis of changes in the magnetic field, and (4) allowing the non-magnetic particles to fall by gravity at the conveyer start edge portion 11 of the belt conveyer B and carrying the ferromagnetic particles in the state of being attracted and held by the belt conveyer B to discharge in the conveyer end edge portion 12 of the belt conveyer B. As shown in Fig. 2, the ferromagnetic particles can be magnetically separated from the powder and granular material a efficiently, even if the thickness of the powder and granular material a supplied to the conveyer belt 1 is large. That is, the ferromagnetic particles can be magnetically separated from the powder and granular material a efficiently and quickly.

In this regard, in the apparatus according to the first embodiment shown in Fig. 2, the magnet roll 4r is rotated and, thereby, 100 times or more in number of changes in the strength and the direction of the magnetic field are given easily while the powder and granular material a is carried along the belt guide roll 3 of the belt conveyer B. In addition, the behavior of the ferromagnetic particles in the magnetic field is changed depending on the powder and granular material a concerned, so that the number of revolutions per minute of the magnet roll 4r can be adjusted to obtain appropriate performance.

Even the apparatus in the related conventional art, as shown in Fig. 8, exerts an effect of separating the ferromagnetic particles in the powder and granular material a because there are changes in the strength and the direction of the magnetic field corresponding to the number of magnets. However, there is a limit to the number of changes in the magnetic field (several times to ten-odd times) because of stationary magnets, and the effects of separating the ferromagnetic particles is small. On the other hand, in the apparatus according to the present first embodiment, the magnet roll 4r is rotated and, therefore, 100 times or more in number of changes in the magnetic field are given easily while the powder and granular material is carried along the conveyer belt 2.

As described above, the magnetic separator according to the present first embodiment can magnetically separate the ferromagnetic particles from the powder and granular material a efficiently. Therefore, in magnetic separation of the powder and granular material a by using this apparatus, as shown in Fig. 2, it is desirable that the powder and granular material be supplied from the supply device 6 to the conveyer belt 1 of the belt conveyer A with a layer thickness larger than the diameter of the smallest particle contained in the powder and granular material a and, in addition, with a layer thickness which allows the magnetic force to act sufficiently. Specifically, the thickness of the powder and granular material may be 20 to 30 mm.

The powder and granular material which is the object of magnetic separation by the apparatus according to the present first embodiment is not specifically limited. Examples thereof include slag, e.g., ironmaking slag, and tailing ores. Among them, in particular, application to the magnetic separation of slag is favorable.

In the iron content recovery from the slag, initially, the ironmaking slag is micronized. If the micronization is insufficient, the recovery rate of the iron content is not improved. There are various steps in the ironmaking and steelmaking processes to generate the ironmaking slag, so that various types of slags are generated. The slag particle diameter after the micronization is determined depending on the slag. In many cases, micronization to several tens of micrometers to about 1 millimeter is required depending on the form of iron contained. The common method for micronization is crushing. Crushing with a jaw crusher or a hammer crusher is performed as rough crushing and, thereafter, crushing is performed by using a ball mill, a rod mill, a jet mill, a pin mill, an impact mill, or the like for the purpose of micronization. As for another method, a method in which heating to about 1,000°C to 1,300°C is performed and, thereafter, cooling is performed gradually is also mentioned.

Then, magnetic separation is performed by the magnetic separator according to the present invention, where the object is the micronized slag. The iron content can be separated and recovered from the slag efficiently by the present invention.

In the first embodiment shown in Fig. 2, magnets 5 are disposed over the width direction of the belt guide roll 3 (magnet roll 4r) in such a way that the magnetic poles of the portion facing the powder and granular material a become the same. In the case where the same magnetic poles are arranged in the width direction, a uniform magnetic field is formed and a force acted on the ferromagnetic particles becomes uniform. However, if the magnets 5 are arranged in such a way that the magnetic poles are different in the width direction, the magnetic field becomes nonuniform and portions, where ferromagnetic particles are not separated, result locally, so that the separation efficiency is reduced.

The members around the rotating magnet roll are influenced by an eddy-current effect due to the changing magnetic field, and metal members, which are even non-magnetic materials, are heated by the eddy current. Consequently, the conveyer belt 2 and the belt guide roll 3 of the belt conveyer B according to the present embodiment are formed from nonmetal, e.g., resin or ceramics.

The apparatus according to the present first embodiment separates the ferromagnetic particles by allowing the magnetic field of the magnet roll 4r disposed inside the belt guide roll 3 on the conveyer start edge portion 11 side of the belt conveyer B to act on the powder and granular material a (powder and granular material layer) carried with the belt conveyer A and attracting and moving the ferromagnetic particles in the powder and granular material a to the lower surface side of the belt conveyer B. Therefore, the distance between the conveyer end edge portion 10 of the belt conveyer A and the conveyer start edge portion 11 of the belt conveyer B may be a dimension at which the magnetic force of the magnet roll 4r acts on the ferromagnetic particles in the powder and granular material a sufficiently. In general, the dimension at which the upper surface of the layer of the powder and granular material a carried with the conveyer belt 1 of the belt conveyer A comes into contact with the conveyer start edge portion 11 of the belt conveyer B, that is, the powder and granular material layer can be slipped between the conveyer end edge portion 10 of the belt conveyer A and the conveyer start edge portion 11 of the belt conveyer B, is preferable.

Next, the modified example 1 of the first embodiment according to the present invention will be described. Fig. 4 is a diagram showing a magnetic separator according to the modified example 1 of the the first embodiment of the present invention.

In the modified example 1, the positional relationship between the belt conveyer A and the belt conveyer B is specified to be a form different from the form shown in Fig. 2. That is, the conveyer start edge portion 11 of the belt conveyer B is closely located above the conveyer end edge portion 10 of the belt conveyer A, and the belt guide rolls 8 and 9 of the belt conveyer A and the belt guide rolls 3 and 13 of the belt conveyer B are rotated in the same direction. Meanwhile, the conveyer belts 1 and 2 are moved in the directions reverse to each other in the conveyer end edge portion 10 of the belt conveyer A and the conveyer start edge portion 11 of the belt conveyer B.

As a matter of course, even in the case where such an arrangement is employed, the ferromagnetic particles can be separated. In this regard, the configuration other than the positional relationship between the belt conveyers A and B is substantially the same as the configuration of the first embodiment shown in Figs. 2 and 3 and, therefore, the explanations thereof will not be provided.

Next, the modified example 2 of the first embodiment according to the present invention will be described. Fig. 5 is an explanatory diagram showing the modified example 2 of the magnetic separator according to the first embodiment of the present invention and a magnetic separation method by using this apparatus.

In the modified example 2 of the first embodiment, the belt guide roll 3 is formed from a sleeve body with a hollow inside and is rotatably supported. A magnetic field application device 4 provided with a plurality of magnets 5, which are arranged at a predetermined interval along the roll circumferential direction, is disposed inside the belt guide roll 3.

The magnetic field application device 4 in the modified example 2 is not rotated in contrast to the magnet roll 4r in the first embodiment. Put another way, the magnets 5 of the magnetic field application device 4 are disposed independently of the belt guide roll 3 and are stationary magnets which are not rotated. In this regard, as shown in Fig. 3, the magnets 5 of the magnetic field application device 4 are arranged in such a way that the magnetic poles adjacent in the roll circumferential direction are different from each other and, in addition, are arranged in such a way that the magnetic poles adjacent in the roll width direction are the same.

As shown in Fig. 5, in the modified example 2 of the first embodiment, the range of disposition of the magnets 5 in the roll circumferential direction is the range of at least about 180° (one-half the circumference of the belt guide roll 3) which is from the lower edge portion of the belt guide roll 3 (the position facing the conveyer end edge portion 10 of the belt conveyer A) to the top position of the belt guide roll 3. The range of disposition of the magnets 5 can be reduced by disposing the magnets 5 in such a way that the magnets 5 are fixed and are not rotated, as in the modified example 2.

In the magnetic separator according to the modified example 2, the ferromagnetic particles in the powder and granular material a are attracted by the magnetic field application device 4 provided with stationary magnets 5, and the powder and granular material a (or part thereof) having the form, in which the ferromagnetic particles enclose non-magnetic particles, is attached to (held by) the lower surface side of the belt conveyer B and are carried with the conveyer belt 2. In this apparatus as well, although the effect is small as compared with the effect of the magnet roll 4r shown in Fig. 2, the ferromagnetic particles in the powder and granular material a undergo action of the magnetic force of the magnets 5 included in the magnetic field application device 4 and the magnetic field is switched in the manner of strong → weak → strong → weak → ··· during carrying with the conveyer belt 2. Consequently, the manner of gathering → dispersion → gathering → dispersion → ··· is repeated with respect to the ferromagnetic particles in the powder and granular material a, so that the same quality of effect as with the first embodiment shown in Fig. 2 is obtained. However, the magnetic field does not change at a high speed in contrast to the magnet roll 4r shown in Fig. 2 and, therefore, the magnetic separability and the treatment speed are low as compared with those in the first embodiment shown in Fig. 2.

The magnetic separator according to the modified example 2 has operation advantages, such as, (i) in the adopted basic system, the magnetic field by the magnetic field application device 4 included in the second belt conveyer B is acted on the powder and granular material a, which is discharged from the first belt conveyer A, from above to attract the ferromagnetic material contained in the powder and granular material a and move to the belt conveyer B side, so that enclosure and entanglement of the non-magnetic particles by the ferromagnetic particles can be reduced as compared with those of the apparatus in the related conventional art and, in addition, (ii) entanglement and enclosure of the non-magnetic particles by the ferromagnetic particles are resolved on the basis of changes in the magnetic field by the magnetic field application device 4.

Fig. 6 is a perspective view showing the structure of a belt guide roll of a modified example 3 of the magnetic separator according to the first embodiment shown in Fig. 2. As shown in Fig. 6, in the modified example 3 of the first embodiment, magnets 5 are included in the magnet roll 4r, where a plurality of magnets 5 are disposed in the circumferential direction of the belt guide roll 3 (magnet roll 4r) and only one magnet 5 is disposed in the width direction of the belt guide roll 3 (magnet roll 4r). The magnets 5 are arranged in such a way that the magnetic poles facing the powder and granular material a come into alternate sequence along the circumferential direction. The magnets 5 may have the above-described configuration.

### [Embodiment not covered by the claimed invention]

Fig. 7 is an explanatory diagram showing an embodiment of a magnetic separator not covered by the claimed invention and a magnetic separation method by using this apparatus.

The magnetic separator according to the embodiment not covered by the claimed invention is a belt conveyer style magnetic separator as with the first embodiment. The magnetic separator according to the embodiment not covered by the claimed invention supplies a powder and granular material (a) containing ferromagnetic particles from a supply device to a conveyer belt 201 and attracts and separates the ferromagnetic particles, by a magnetic force, from non-magnetic particles when the powder and granular material a is discharged from a conveyer end edge portion 2010.

In Fig. 7, reference numeral 201 denotes a conveyer belt, reference numeral 202 denotes a belt guide roll on the conveyer end edge portion 2010 side, and reference numeral 208 denotes a belt guide roll on the conveyer start edge portion 2011 side. The conveyer belt 201 is disposed between the belt guide rolls 202 and 208 and, thereby, the belt conveyer is formed. The belt guide roll 208 is driven by a drive device, e.g., a motor, and thereby, the conveyer belt 201 is rotated in the belt conveyer. The belt guide roll 202 is a non-driven roll and is formed from a sleeve body with a hollow inside.

A magnet roll 203 is disposed inside the belt guide roll 202. The configuration of the magnet roll 203 is substantially the same as the configuration shown in Fig. 3. Specifically, the magnet roll 203 is provided with a plurality of magnets 205 arranged in the circumference direction and the width direction thereof at predetermined intervals and, in addition, the magnetic poles of the magnets 205 adjacent in the roll circumferential direction are different magnetic poles (north pole, south pole). That is, magnets 205 are arranged in such a way that the north poles and the south poles are arranged alternately in the roll circumference direction. The plurality of magnets 205 are arranged in such a way that the same magnetic poles are aligned in the roll width direction.

The magnet roll 203 is a roll rotated by a motor or the like and is rotated in the direction reverse to the direction of the belt guide roll 202. Also, as described later, this magnet roll 203 is rotated at a speed higher than the speed of the belt guide roll 202.

The members around the rotating magnet roll are influenced by an eddy-current effect due to the changing magnetic field, and metal members, which are even non-magnetic materials, are heated by the eddy current. Consequently, the conveyer belt 201 and the belt guide roll 202 are formed from a nonmetal, e.g., a resin or ceramics.

The magnets 205 are arranged in such a way that the magnetic poles become the same over the width direction of the magnet roll 203. In the case where the same magnetic poles are arranged in the width direction, a uniform magnetic field is formed and a force acted on the ferromagnetic particles becomes uniform. However, if the magnets 205 are arranged in such a way that the magnetic poles are different in the width direction, the magnetic field becomes nonuniform and portions, where ferromagnetic particles are not separated, result locally, so that the separation efficiency is reduced. In this regard, as for the magnet 205, one magnet may be disposed in the width direction, as shown in Fig. 6, or appropriately divided magnets may be disposed, as shown in Fig. 3.

The number of magnets 205 arranged along the outer circumference of the magnet roll 203, the arrangement interval, and the like are not specifically limited. High-speed changes in the magnetic field are obtained even when the rotational speed is low by increasing the number of the magnets 205 or reducing the arrangement interval.

In the embodiment not covered by the claimed invention , as with the first embodiment, it is preferable that changes in the strength and the direction of the magnetic field be allowed to occur at a maximized speed. Specifically, the magnetic field change frequency F (Hz), which is defined by the following formula (1), of the magnet roll 203 is preferably 170 Hz or more. The magnetic field change frequency is more preferably 200 Hz or more.$F = \left(x⋅P\right) / 60$ where x: the number of revolutions per minute of magnet roll (rpm)
P: the number of magnetic poles provided to magnet roll (in this regard, as for the number of magnetic poles, a pair of the north pole and the south pole adjacent in the circumferential direction of the surface facing the powder and granular material (a) of the magnet roll 203 is counted as one magnetic pole and, for example, in the case where the north pole [a], the south pole [b], and the north pole [c] are aligned in the circumferential direction, the pair of the north pole [a] and the south pole [b] is counted as one magnetic pole and the pair of the south pole [b] and the north pole [c] is counted as one magnetic pole)

For example, in the case where 12 poles (a pair of the north pole and the south pole is counted as one magnetic pole) of magnets (for example, neodymium magnets) are disposed in the circumferential direction, when the rotational speed of the magnet roll 203 is specified to be 1,000 rpm, the magnetic field change frequency results in 200 Hz. In the case where 24 poles (a pair of the north pole and the south pole is counted as one magnetic pole) of magnets are disposed in the circumferential direction and the magnetic field change frequency is specified to be 200 Hz likewise, the rotational speed of the magnet roll 203 may be 500 rpm.

The upper limit of the magnetic field change frequency is about 1,000 Hz because there is a mechanical upper limit to the number of revolutions per minute of the magnet roll 203 and the effect of changes in the magnetic field may be saturated even when the frequency is increased.

The size of the magnet 205 is not specifically limited insofar as the size is suitable for arranging the predetermined number of magnets. The strength of the magnetic field due to the magnets 205 is not specifically limited. Usually, the magnets 205 are selected in such a way that about 0.01 to 0.5 T is ensured in the conveyer belt portion in contact with the belt guide roll 202 in accordance with an object. If the magnetic field is too weak, the effect of the magnet roll 203 is not obtained sufficiently. On the other hand, if the magnetic field is too strong, the attractive force acted on the ferromagnetic particles is too strong and separation of the ferromagnetic particles on the basis of the above-described principle (Fig. 1 (A) to (D)) may be hindered conversely.

In the apparatus according to the embodiment not covered by the claimed invention as well, the basic function of separating the ferromagnetic particles is the same as that described with reference to Fig. 1.

It is the feature that when the magnet roll 203 is rotated, the magnetic field is switched in the manner of strong → weak → strong → weak → ··· instantaneously and the effect on the ferromagnetic particles in the powder and granular material layer is repeated in the manner of gathering → dispersion → gathering → dispersion → ··· because of the plurality of magnets 205 arranged at the predetermined interval and the space portions between adjacent magnets 205. The width of space portions between adjacent magnets 205 in the roll circumferential direction is not specifically limited, although about 1 to 50 mm is appropriate in order that the state in which the ferromagnetic particles in the powder and granular material layer are released from the magnetic field occurs appropriately, whereas the state in which the magnetic field is weakened does not continue for a long time.

A partition plate 206 is disposed below (just below) the belt guide roll 202 and along the conveyer belt width direction. In addition, a clearance S for allowing the passage of the ferromagnetic particles is disposed between the upper edge portion of the partition plate 206 and the conveyer belt 201 (conveyer belt portion with the movement direction reversed by the belt guide roll 202). The partition plate 206 is disposed in such a form for the purpose of avoiding mixing of the non-magnetic particles with the ferromagnetic particles during falling because the fall area of the non-magnetic particles and the fall area of the ferromagnetic particles are adjacent to each other.

Also, a magnetically attracted material recovery portion 207x and a magnetically not-attracted material recovery portion 207y are disposed at positions sandwiching the partition plate 206 in the conveyer belt movement direction. That is, the magnetically attracted material recovery portion 207x is disposed at the position on the conveyer start edge portion 2011 side (fall area of the ferromagnetic particles) and the magnetically not-attracted material recovery portion 207y is disposed on the position of the conveyer end edge portion 2010 side (fall area of the non-magnetic particles), while the partition plate 206 is sandwiched between them.

The function and the operation of the magnetic separator according to the embodiment not covered by the claimed invention and the magnetic separation method by using this apparatus will be described below.

In the magnetic separator according to the embodiment not covered by the claimed invention , the belt feed speed of the conveyer belt 201 (rotational speeds of the belt guide rolls 202 and 208) may be specified to be a speed required for the treatment process. The rotational speed of the magnet roll 203 is determined in such a way that the speed of changes in the magnetic field become sufficiently high relative to this belt feed speed. In particular, it is preferable that the rotational speed of the magnet roll 203 be set in such a way as to satisfy the above-described condition represented by the formula (1).

A sufficient thickness of powder and granular material a containing the ferromagnetic particles is supplied from a supply device 204 to the conveyer belt 201 in operation and is carried to the conveyer end edge portion 2010 (positions of the belt guide roll 202 and the magnet roll 203). Then, when the powder and granular material a on the conveyer belt 201 is discharged from the conveyer end edge portion 2010, the ferromagnetic particles in the powder and granular material a undergo action of the magnetic field of the magnets 205 included in the magnet roll 203 and the strength of the magnetic field is switched in the manner of strong → weak → strong → weak → ··· instantaneously because of the rotation of the magnet roll 203. The effect in the manner of gathering → dispersion → gathering → dispersion → ··· is repeated on the ferromagnetic particles in the powder and granular material a.

In the conveyer end edge portion 2010, the powder and granular material a is fed along the arc of the belt guide roll 202 in association with the movement of the conveyer belt 201, and the non-magnetic particles fall freely by gravity in a region of one-quarter turn to one-half turn. On the other hand, the mass of the ferromagnetic particles is reduced because of micronization, and the strength of the magnetic field is sufficiently high. Therefore, the ferromagnetic particles are attracted by the magnet immediately on the occasion of fall from the conveyer belt 201. Consequently, the ferromagnetic particles are fed in the movement direction of the conveyer belt 201 and fall freely outside the magnetic field area after one-half turn or more. Subsequently, the non-magnetic particles which fall first are recovered into the magnetically not-attracted material recovery portion 207y and the ferromagnetic particles which fall thereafter are recovered into the magnetically attracted material recovery portion 207x. At this time, mixing of the non-magnetic particles with the ferromagnetic particles is prevented by the partition plate 206. In this regard, the position of the partition plate 206 may be adjusted in accordance with the feed speed of the conveyer belt 201 and the falling behavior of the powder and granular material a.

In the magnetic separator according to the embodiment not covered by the claimed invention , magnets 205 are disposed over the width direction of the belt guide roll 202 (magnet roll 203) in such a way that the magnetic poles facing the powder and granular material a become the same. Consequently, there are advantages that a uniform magnetic field is formed in the width direction and the magnetic force acted on the ferromagnetic particles becomes uniform.

Also, in the magnetic separator according to the embodiment not covered by the claimed invention , the ferromagnetic particles can be efficiently magnetically separated even when the layer thickness of the powder and granular material a supplied to the conveyer belt 201 is sufficiently increased, as shown in Fig. 7, because of the functions of (i) mechanically generating high-speed changes in the magnetic field by rotating the magnet roll 203, (ii) supplying the powder and granular material a with a sufficient layer thickness into the resulting changing magnetic field, (iii) moving the ferromagnetic particles to the magnet roll 203 side and excluding the non-magnetic particles to the side apart from the magnet roll 203 while entanglement and enclosure of the non-magnetic particles by the ferromagnetic particles are resolved on the basis of changes in the magnetic field, and (iv) allowing the non-magnetic particles to fall by gravity below the belt guide roll 202 and carrying the ferromagnetic particles in the state of being attracted and held on the conveyer belt 201 side to allow the ferromagnetic particles to fall when the effect of the magnetic field disappear. That is, the ferromagnetic particles can be magnetically separated from the powder and granular material a efficiently and quickly.

Even the apparatus in the related conventional art, as shown in Fig. 8, exerts an effect of separating the ferromagnetic particles in the powder and granular material a because there are changes in the strength and the direction of the magnetic field corresponding to the number of magnets. However, there is a limit to the number of changes in the magnetic field (several times to ten-odd times) because of stationary magnets, and the effects of separating the ferromagnetic particles is small. On the other hand, in the apparatus according to the embodiment not covered by the claimed invention, the magnet roll 203 is rotated and, therefore, 100 times or more in number of changes in the magnetic field are given easily while the powder and granular material a is carried along the belt guide roll 202.

In addition, the agitation behavior changes depending on the powder and granular material a, so that the number of revolutions per minute of the magnet roll 203 can be adjusted in such a way that appropriate performance is obtained.

As described above, the magnetic separator according to the embodiment not covered by the claimed invention can magnetically separate the ferromagnetic particles from the powder and granular material a efficiently. Therefore, in magnetic separation of the powder and granular material a by using this apparatus, as shown in Fig. 7, it is desirable that the powder and granular material be supplied from the supply device 204 to the conveyer belt 201 with a layer thickness larger than the diameter of the smallest particle contained in the powder and granular material a and, in addition, with a layer thickness which allows the magnetic force to act sufficiently. Specifically, the thickness of the powder and granular material may be 20 to 30 mm.

Also, it is preferable that the clearance S between the upper edge portion of the partition plate 206 and the conveyer belt 201 be smaller than the layer thickness of the powder and granular material a supplied from the supply device 204 to the conveyer belt 201. The purpose of disposition of the partition plate 206 is as described above. In order to prevent mixing of the ferromagnetic particles falling from the conveyer belt 201 in the conveyer end edge portion 2010 with the non-magnetic particles, it is desirable that the upper edge portion of the partition plate 206 be brought close to the conveyer belt 201 as much as possible. Specifically, mixing of the ferromagnetic particles with the non-magnetic particles can be prevented by specifying the clearance S to be smaller than the layer thickness of the powder and granular material a.

The powder and granular material which is the object of magnetic separation by the apparatus according to the embodiment not covered by the claimed invention is not specifically limited. Examples thereof include slag, e.g., ironmaking slag, and tailing ores. Among them, in particular, application to the magnetic separation of slag is favorable.

In the iron content recovery from the slag, initially, the ironmaking slag is micronized. If the micronization is insufficient, the recovery rate of the iron content is not improved. There are various steps in the ironmaking and steelmaking processes to generate the ironmaking slag, so that various types of slags are generated. The slag particle diameter after the micronization is determined depending on the slag. In many cases, micronization to several tens of micrometers to about 1 millimeter is required depending on the form of iron contained. The common method for micronization is crushing. Crushing with a jaw crusher or a hammer crusher is performed as rough crushing and, thereafter, crushing is performed by using a ball mill, a rod mill, a jet mill, a pin mill, an impact mill, or the like for the purpose of micronization. As for another method, a method in which heating to about 1,000°C to 1,300°C is performed and, thereafter, cooling is performed gradually is also mentioned. Then, magnetic separation is performed by the magnetic separator not covered by the claimed invention, where the object is the micronized slag. Consequently, the iron content can be separated and recovered from the slag efficiently, and the productivity of a slag treatment line can be enhanced.

Meanwhile, as for the separator of the ferromagnetic particles, an eddy-current style separator having a seemingly similar structure is known. However, there is a difference in the principle of separation of metal particles. In addition, particles are splashed by repulsion and, therefore, a mechanism to adjust the position of a recovery case in accordance with the size of the metal particles to be recovered is necessary and a space therefor is also necessary. On the other hand, in the present invention, such positional adjustment of the recovery case is unnecessary, so that a complicated mechanism therefor is unnecessary.

In this regard, the present invention is not limited to the magnetic separator and magnetic separation method according to the above-described first embodiment, and various design changes can be performed , as long as they fall within the scope of the appended claims Also, execution as a method for producing an iron source to produce the iron source from a by-product of the ironmaking process is possible by using the magnetic separation method according to the first embodiment.

### [EXAMPLE 1]

Magnetic separation of a steelmaking slag was performed by using the magnetic separator according to the first embodiment of the present invention, as shown in Fig. 2.

A crushed material of a steelmaking slag was sifted through a 400-µm sieve and, thereafter, the slag passed through the mesh of the sieve was taken as an object powder and granular material of magnetic separation. The iron concentration in this powder and granular material was 54 percent by mass. The supply layer thickness of the powder and granular material on the conveyer belt 1 of the belt conveyer A was specified to be 7 mm. The outside diameter of the belt guide roll 3 of the belt conveyer B was 300 mm, the number of magnetic poles of the magnet roll 4r was 12 poles (where the pair of the north pole and the south pole was specified to be one magnetic pole), the feed speeds of the conveyer belts 1 and 2 of the belt conveyers A and B were 0.5 m/sec., the rotational speed of the belt guide roll 3 was 31.9 rpm, and the magnetic field strength in the conveyer belt portion in contact with the belt guide roll 3 was 0.2 T. Also, in order to examine the effect of the rotational speed of the magnet roll 4r of the belt conveyer B, the rotational speed of the magnet roll 4r was specified to be 500 rpm (magnetic field change frequency F = 100 Hz), 850 rpm (magnetic field change frequency F = 170 Hz), or 1,200 rpm (magnetic field change frequency F = 240 Hz).

For purposes of comparison, same powder and granular material of the same steelmaking slag was magnetically separated by using a magnetic drum separator A (the magnetic field strength on the drum surface: 0.16 T) and a magnetic pulley B (the magnetic field strength in the conveyer belt portion in contact with the belt guide roll: 0.2 T) commonly used in the related conventional art at a feed speed of 0.5 m/sec.

In each of the above-described examples, the iron concentration in a magnetic attraction recovered material and the iron recovery rate from the slag were examined. The results thereof are shown in Table 1.

To begin with, as for the magnetic attraction recovered material of Comparative example 1 in which the magnetic drum separator A was used, the iron concentration was low because a nonferrous component is entangled and the iron recovery rate was also low because iron was released to the magnetically not-attracted side. Meanwhile, as for Comparative example 2 in which the magnetic pulley B was used, almost all amount of powder and granular material was entangled and, therefore, the iron recovery rate was certainly good, although an important iron concentration in the magnetic attraction recovered material was substantially the same as that of the powder and granular material before magnetic separation. On the other hand, as for the present invention example, in the case where the magnetic field change frequency of the magnet roll 4r was specified to be 170 Hz or more, both the iron concentration in the magnetic attraction recovered material and the iron recovery rate from the slag took on high values. Furthermore, in the case where the magnetic field change frequency of the magnet roll 4r was specified to be 200 Hz or more, both the iron concentration in the magnetic attraction recovered material and the iron recovery rate from the slag took on higher values.

**[Table 1]**

| | | Iron concentration in magnetic attraction recovered material | Iron recovery rate from slag |
|---|---|---|---|
| Comparative example 1: magnetic drum separator A (0.16 T) | | 62 mass% | 82 mass% |
| Comparative example 2: magnetic pulley B (0.2 T) | | 55 mass% | 99 mass% |
| Invention example: (change in magnetic field 0.2 T) | Number of revolutions per minute of magnet roll = 500 rpm | 72 mass% | 78 mass% |
| | Number of revolutions per minute of magnet roll = 850 rpm | 80 mass% | 85 mass% |
| | Number of revolutions per minute of magnet roll = 1200 rpm | 92 mass% | 95 mass% |

### [EXAMPLE 2]

Magnetic separation of a steelmaking slag was performed by using the magnetic separator according to the embodiment not covered by the claimed invention , as shown in Fig. 7.

A crushed material of a steelmaking slag was sifted through a 400-µm sieve and, thereafter, the slag passed through the mesh of the sieve was taken as an object powder and granular material of magnetic separation. The iron concentration in this powder and granular material was 54 percent by mass. The supply layer thickness of the powder and granular material on the conveyer belt 201 was specified to be 7 mm. The outside diameter of the belt guide roll 202 was 300 mm, the number of magnetic poles of the magnet roll 203 was 12 poles (where the pair of the north pole and the south pole was specified to be one magnetic pole), the feed speed of the conveyer belt 201 was 0.5 m/sec., the rotational speed of the belt guide roll 202 was 31.9 rpm, and the magnetic field strength in the conveyer belt portion in contact with the belt guide roll 202 was 0.2 T. Also, in order to examine the effect of the rotational speed of the magnet roll 203, the rotational speed of the magnet roll 203 was specified to be 500 rpm (magnetic field change frequency F = 100 Hz), 850 rpm (magnetic field change frequency F = 170 Hz), or 1,200 rpm (magnetic field change frequency F = 240 Hz).

For purposes of comparison, same powder and granular material of the same steelmaking slag was magnetically separated by using a magnetic drum separator A (the magnetic field strength on the drum surface: 0.16 T) and a magnetic pulley B (the magnetic field strength in the conveyer belt portion in contact with the belt guide roll 202: 0.2 T) commonly used in the related conventional art at a feed speed of 0.5 m/sec.

In each of the above-described examples, the iron concentration in a magnetic attraction recovered material and the iron recovery rate from the slag were examined. The results thereof are shown in Table 2.

To begin with, as for the magnetic attraction recovered material of Comparative example 1 in which the magnetic drum separator A was used, the iron concentration was low because a nonferrous component is entangled and the iron recovery rate was also low because iron was released to the magnetically not-attracted side. Meanwhile, as for Comparative example 2 in which the magnetic pulley B was used, almost all amount of powder and granular material was entangled and, therefore, the iron recovery rate was certainly good, although an important iron concentration in the magnetic attraction recovered material was substantially the same as that in the powder and granular material before magnetic separation. On the other hand, as for the present invention example, in the case where the magnetic field change frequency of the magnet roll 203 was specified to be 170 Hz or more, both the iron concentration in the magnetic attraction recovered material and the iron recovery rate from the slag took on high values. Furthermore, in the case where the magnetic field change frequency of the magnet roll 203 was specified to be 200 Hz or more, both the iron concentration in the magnetic attraction recovered material and the iron recovery rate from the slag took on higher values.

**[Table 2]**

| | | Iron concentration in magnetic attraction recovered material | Iron recovery rate from slag |
|---|---|---|---|
| Comparative example 1: magnetic drum separator A (0.16 T) | | 62 mass% | 82 mass% |
| Comparative example 2: magnetic pulley B (0.2 T) | | 55 mass% | 99 mass% |
| Invention example: (change in magnetic field 0.2 T) | Number of revolutions per minute of magnet roll = 500 rpm | 68 mass% | 70 mass% |
| | Number of revolutions per minute of magnet roll = 850 rpm | 77 mass% | 81 mass% |
| | Number of revolutions per minute of | 89 mass% | 94 mass% |
| | magnet roll = 1200 rpm | | |

### [Reference Signs List]

1, 2, 20 conveyer belt
3, 8, 9, 13 belt guide roll
4 magnetic field application device
4r magnet roll
5 magnetic pole, magnet
6 supply device
7x magnetically attracted material recovery portion
7y magnetically not-attracted material recovery portion
10, 12 conveyer end edge portion
11, 14 conveyer start edge portion
15 bearing
21 belt guid roll
22 magnet
23 supply device
24x magnetically attracted material recovery portion
24y magnetically not-attracted material recovery portion
25 partition plate
26 vibration feeder
27 conveyer end edge portion
30, 40 roll shaft
A, B belt conveyer
a powder and granular material
201 conveyer belt
202 belt guide roll
203 magnet roll
204 supply device
205 magnetic pole, magnet
206 partition plate
207x magnetically attracted material recovery portion
207y magnetically not-attracted material recovery portion
208 belt guide roll
2010 conveyer end edge portion
2011 conveyer start edge portion
S clearance

## Claims

1. A magnetic separator comprising:
a conveyer belt (2) of a second belt conveyer (B) to carry a powder and granular material (a) containing ferromagnetic particles:
a rotatable hollow belt guide roll (3) having an outer circumference partly wound with the above-described conveyer belt (2); and
a magnetic field application device (4) disposed inside the belt guide roll (3),
a first belt conveyer (A) to carry the powder and granular material (a) containing ferromagnetic particles; and
the second belt conveyer (B) provided with the magnetic field application device (4) and located above the first belt conveyer (A), and
wherein the magnetic field application device (4) includes a plurality of magnets (5) inside the belt guide roll (3),
the magnets (5) are arranged in such a way that magnetic poles adjacent in the circumferential direction of the belt guide roll (3) are different from each other,
the powder and granular material (a) containing ferromagnetic particles is supplied to the first belt conveyer (A) from a supply device (6),
a conveyer start edge portion (11) of the second belt conveyer (B) is closely located above a conveyer end edge portion (10) of the first belt conveyer (A), and
a magnetically attracted material recovery portion (7x) is disposed below the conveyer end edge portion (12) of the second belt conveyer (B) and a magnetically not-attracted material recovery portion (7y) is disposed below the conveyer start edge portion (11) of the second belt conveyer (B), and wherein
the conveyer start edge portion (11) of the second belt conveyer (B) is a portion in which the powder and granular material (a) containing ferromagnetic particles starts to contact with the second belt conveyer (B) and the conveyer end edge portion (12) of the second belt conveyer (B) is a portion in which the powder and granular material (a) containing ferromagnetic particles is discharged from the second belt conveyer (B),
wherein the conveyer end edge portion (10) of the first belt conveyer (A) is a portion where the powder and granular material (a) slips between the conveyer end edge portion (10) of the first belt conveyer (A) and the conveyer start edge portion (11) of the second belt conveyer (B), and wherein
the magnetic field change frequency F in Hz, which is defined by the following formula (1) and which indicates changes in the magnetic field acted on the powder and granular material (a) from the magnetic field application device (4), is 170 Hz or more, $F = \left(x⋅P\right) / 60$ where x: the number of revolutions per minute of a magnet roll (4r)
P: the number of magnetic poles (5) provided to the magnet roll (4r), wherein, as for the number of magnetic poles (5), a pair of the north pole and the south pole adjacent in the circumferential direction of the surface facing the powder and granular material (a) of the magnet roll (4r) is counted as one magnetic pole.

2. The magnetic separator according to Claim 1, wherein
the magnets (5) are arranged in such a way that adjacent magnetic poles (N, S) in the width direction of the belt guide roll are the same.

3. The magnetic separator according to any one of the preceding claims, comprising:
the magnetic field application device (4) provided with a plurality of magnetic poles (5) arranged along the roll circumferential direction at a predetermined interval, where magnetic poles (5) adjacent in the roll circumferential direction are different from each other, is disposed inside the belt guide roll (3) at the conveyer start edge portion (11) side of the second belt conveyer (B).

4. The magnetic separator according to any one of the preceding Claims,
wherein the magnetic field application device (4) of the second belt conveyer (B) is formed from the magnet roll (4r) driven to rotate, and
the conveyer belt (2) and the belt guide roll (3) of the second belt conveyer (B) are made from a non-metal and, in addition, the belt guide roll (3) is specified to be a nondriven roll.

5. A magnetic separation method comprising the steps of:
using the magnetic separator according to any one of the preceding Claims, and
supplying a powder and granular material (a) from a supply device (6) to the first belt conveyer (A) with a layer thickness larger than the diameter of the smallest particle contained in the powder and granular material (a), and wherein
the magnetic field change frequency F in Hz, which is defined by the following formula (1), of the magnet roll (4r) is specified to be 170 Hz or more, $F = \left(x⋅P\right) / 60$
where x: the number of revolutions per minute of magnet roll (4r)
P: the number of magnetic poles (5) provided to magnet roll (4r), wherein a pair of the north pole and the south pole is counted as one magnetic pole.

6. The magnetic separation method according to Claim 5, wherein the conveyer belt (1) of the first belt conveyer (A) and the conveyer belt (2) of the second belt conveyer(B) are moved in the same directions or in the directions reverse to each other in the conveyer end edge portion (10) of the first belt conveyer (A) and the conveyer start edge portion (11) of the second belt conveyer (B).

7. A method for manufacturing an iron source to produce the iron source from a by-product of an ironmaking process, comprising the step of using the magnetic separator according to any of Claims 1 to 4 or the magnetic separation method according to Claim 5 or 6.

## Patentansprüche

1. Magnetabscheider, der umfasst:
ein Förderband (2) eines zweiten Bandförderers (B) zum Transportieren eines pulverförmigen und körnigen Materials (a), das ferromagnetische Teilchen enthält;
eine drehbare hohle Bandführungsrolle (3), die einen Außenumfang hat, der teilweise mit dem oben beschriebenen Förderband (2) umwickelt ist; sowie
eine Vorrichtung (4) zum Anlegen eines Magnetfeldes, die im Inneren der Bandführungsrolle (3) angeordnet ist,
einen ersten Bandförderer (A) zum Transportieren des pulverförmigen und körnigen Materials (a), das ferromagnetische Teilchen enthält; und
wobei der zweite Bandförderer (B) mit der Vorrichtung (4) zum Anlegen eines Magnetfeldes versehen und oberhalb des ersten Bandförderers (A) angeordnet ist, und
die Vorrichtung (4) zum Anlegen eines Magnetfeldes eine Vielzahl von Magneten (5) im Inneren der Bandführungsrolle (3) enthält,
die Magnete (5) so angeordnet sind, dass in der Umfangsrichtung der Bandführungsrolle (3) benachbarte Magnetpole voneinander verschieden sind,
das pulverförmige und körnige Material (a), das ferromagnetische Teilchen enthält, dem ersten Bandförderer (A) von einer Zuführvorrichtung (6) zugeführt wird,
ein Förderer-Anfangskantenabschnitt (11) des zweiten Bandförderers (B) dicht über einem Förderer-Endkantenabschnitt (10) des ersten Bandförderers (A) angeordnet ist, und
ein magnetisch angezogener Material-Rückgewinnungsabschnitt (7x) unter dem Förderer-Endkantenabschnitt (12) des zweiten Bandförderers (B) angeordnet ist und ein magnetisch nicht angezogener Material-Rückgewinnungsabschnitt (7y) unter dem Förderer-Anfangskantenabschnitt (11) des zweiten Bandförderers (B) angeordnet ist,
und wobei der Förderer-Anfangskantenabschnitt (11) des zweiten Bandförderers (B) ein Abschnitt ist, in dem das pulverförmige und körnige Material (a), das ferromagnetische Teilchen enthält, beginnt, mit dem zweiten Bandförderer (B) in Kontakt zu kommen, und der Förderer-Endkantenabschnitt (12) des zweiten Bandförderers (B) ein Abschnitt ist, in dem das pulverförmige und körnige Material (a), das ferromagnetische Teilchen enthält, von dem zweiten Bandförderer (B) abgeleitet wird,
wobei der Förderer-Endkantenabschnitt (10) des ersten Bandförderers (A) ein Abschnitt ist, in dem das pulverförmige und körnige Material (a) zwischen dem Förderer-Endkantenabschnitt (10) des ersten Bandförderers (A) und dem Förderer-Anfangskantenabschnitt (11) des zweiten Bandförderers (B) gleitet,
und wobei
die Magnetfeld-Änderungsfrequenz F in Hz, die durch die folgende Formel (1) definiert ist und die Änderungen im Magnetfeld anzeigt, das von der Vorrichtung (4) zum Anlegen eines Magnetfeldes auf das pulverförmige und körnige Material (a) einwirkt, 170 Hz oder mehr beträgt, $F = \left(x⋅P\right) / 60$
wobei
x: die Anzahl von Umdrehungen pro Minute einer Magnetrolle (4r),
P: die Anzahl von Magnetpolen (5), die an der Magnetrolle (4r) vorhanden sind,
und dabei hinsichtlich der Anzahl der Magnetpole(5), ein Paar aus dem Nordpol und dem Südpol, die in der Umfangsrichtung der dem pulverförmigen und dem körnigen Material (a) zugewandten Fläche der Magnetrolle (4r) benachbart sind, als ein Magnetpol gezählt wird.

2. Magnetabscheider nach Anspruch 1, wobei die Magnete (5) so angeordnet sind, dass in der Breitenrichtung der Bandführungsrolle benachbarte Magnetpole (N, S) gleich sind.

3. Magnetabscheider nach einem der vorangehenden Ansprüche, der umfasst:
die Vorrichtung (4) zum Anlegen eines Magnetfeldes mit einer Vielzahl von Magnetpolen (5) versehen ist, die entlang der Walzen-Umfangsrichtung in einem vorgegebenen Intervall angeordnet sind, wobei die in der Walzen-Umfangsrichtung benachbarten Magnetpole (5) voneinander verschieden sind, und im Inneren der Bandführungsrolle (3) an der Seite des Förderer-Anfangskantenabschnitts (11) des zweiten Bandförderers (B) angeordnet ist.

4. Magnetabscheider nach einem der vorangehenden Ansprüche,
wobei die Vorrichtung (4) zum Anlegen eines Magnetfeldes des zweiten Bandförderers (B) von der rotierend angetriebenen Magnetrolle (4r) gebildet wird, und
das Förderband (2) sowie die Bandführungsrolle (3) des zweiten Bandförderers (B) aus einem Nichtmetall bestehen und darüber hinaus die Bandführungsrolle (3) als eine nicht angetriebene Rolle vorgegeben ist.

5. Magnetabscheidungsverfahren, das die folgenden Schritte umfasst:
Einsetzen des Magnetabscheiders nach einem der vorangehenden Ansprüche, sowie
Zuführen eines pulverförmigen und körnigen Materials (a) von einer Zuführvorrichtung (6) zu dem ersten Bandförderer (A) mit einer Schichtdicke, die größer ist als der Durchmesser des kleinsten in dem pulverförmigen und körnigen Material (a) enthaltenen Teilchens, und wobei
die durch die folgende Formel (1) definierte Magnetfeld-Änderungsfrequenz F in Hz der Magnetrolle (4r) mit 170 Hz oder mehr vorgegeben ist, $F = \left(x⋅P\right) / 60$
wobei
x: die Anzahl von Umdrehungen pro Minute einer Magnetrolle (4r),
P: die Anzahl von Magnetpolen (5), die an der Magnetrolle (4r) vorhanden sind, wobei ein Paar aus dem Nordpol und dem Südpol als ein Magnetpol gezählt wird.

6. Magnetisches Abscheidungsverfahren nach Anspruch 5, wobei das Förderband (1) des ersten Bandförderers (A) und das Förderband (2) des zweiten Bandförderers (B) in den gleichen Richtungen oder in den zueinander entgegengesetzten Richtungen in dem Förderer-Endkantenabschnitt (10) des ersten Bandförderers (A) und dem Förderer-Anfangskantenabschnitt (11) des zweiten Bandförderers (B) bewegt werden.

7. Verfahren zum Herstellen einer Eisenquelle, mit dem die Eisenquelle aus einem Nebenprodukt eines Eisenherstellungs-Prozesses produziert wird, wobei es den Schritt zum Einsetzen des Magnetabscheiders nach einem der Ansprüche 1 bis 4 oder des Magnetabscheidungsverfahrens nach Anspruch 5 oder 6 umfasst.

## Revendications

1. Séparateur magnétique comprenant :
une courroie transporteuse (2) d'un deuxième transporteur à courroie (B) pour transporter un matériau pulvérulent et granulaire (a) contenant des particules ferromagnétiques :
un rouleau de guidage de courroie creux rotatif (3) ayant une circonférence externe partiellement enroulée avec la courroie transporteuse (2) décrite ci-dessus ; et
un dispositif d'application de champ magnétique (4) disposé à l'intérieur du rouleau de guidage de courroie (3),
un premier transporteur à courroie (A) pour transporter le matériau pulvérulent et granulaire (a) contenant des particules ferromagnétiques ; et
le deuxième transporteur à courroie (B) pourvu du dispositif d'application de champ magnétique (4) et situé au-dessus du premier transporteur à courroie (A), et
dans lequel le dispositif d'application de champ magnétique (4) comprend une pluralité d'aimants (5) à l'intérieur du rouleau de guidage de courroie (3),
les aimants (5) sont agencés de sorte que des pôles magnétiques adjacents dans la direction circonférentielle du rouleau de guidage de courroie (3) soient différents les uns des autres,
le matériau pulvérulent et granulaire (a) contenant des particules ferromagnétiques est fourni au premier transporteur à courroie (A) à partir d'un dispositif d'alimentation (6),
une partie de bord de début de transporteur (11) du deuxième transporteur à courroie (B) est étroitement située au-dessus d'une partie de bord de fin de transporteur (10) du premier transporteur à courroie (A), et
une partie de récupération de matériau magnétiquement attirée (7x) est disposée en dessous de la partie de bord de fin de transporteur (12) du deuxième transporteur à courroie (B) et une partie de récupération de matériau magnétiquement non attirée (7y) est disposée en dessous de la partie de bord de début de transporteur (11) du deuxième transporteur à courroie (B), et dans lequel
la partie de bord de début de transporteur (11) du deuxième transporteur à courroie (B) est une partie dans laquelle le matériau pulvérulent et granulaire (a) contenant des particules ferromagnétiques commence à entrer en contact avec le deuxième transporteur à courroie (B) et la partie de bord de fin de transporteur (12) du deuxième transporteur à courroie (B) est une partie dans laquelle le matériau pulvérulent et granulaire (a) contenant des particules ferromagnétiques est déchargé du deuxième transporteur à courroie (B), dans lequel
la partie de bord de fin de transporteur (10) du premier transporteur à courroie (A) est une partie où le matériau pulvérulent et granulaire (a) glisse entre la partie de bord de fin de transporteur (10) du premier transporteur à courroie (A) et la partie de bord de début de transporteur (11) du deuxième transporteur à courroie (B), et dans lequel
la fréquence de changement de champ magnétique F en Hz, qui est définie par la formule (1) suivante et qui indique des changements du champ magnétique agissant sur le matériau pulvérulent et granulaire (a) depuis le dispositif d'application de champ magnétique (4), est supérieure ou égale à 170 Hz, $F = \left(x⋅P\right) / 60$
où x : le nombre de tours par minute d'un rouleau magnétique (4r)
P : le nombre de pôles magnétiques (5) fournis au rouleau magnétique (4r), dans lequel, en ce qui concerne le nombre de pôles magnétiques (5), une paire du pôle nord et du pôle sud adjacents dans la direction circonférentielle de la surface faisant face au matériau pulvérulent et granulaire (a) du rouleau magnétique (4r) est comptée comme un pôle magnétique.

2. Séparateur magnétique selon la revendication 1, dans lequel
les aimants (5) sont agencés de sorte que des pôles magnétiques adjacents (N, S) dans la direction de largeur du rouleau de guidage de courroie soient identiques.

3. Séparateur magnétique selon l'une quelconque des revendications précédentes, comprenant :
le dispositif d'application de champ magnétique (4) pourvu d'une pluralité de pôles magnétiques (5) agencés le long de la direction circonférentielle de rouleau à un intervalle prédéterminé, où des pôles magnétiques (5) adjacents dans la direction circonférentielle de rouleau sont différents les uns des autres, est disposé à l'intérieur du rouleau de guidage de courroie (3) du côté de la partie de bord de début de transporteur (11) du deuxième transporteur à courroie (B).

4. Séparateur magnétique selon l'une quelconque des revendications précédentes,
dans lequel le dispositif d'application de champ magnétique (4) du deuxième transporteur à courroie (B) est formé à partir du rouleau magnétique (4r) entraîné en rotation, et
la courroie transporteuse (2) et le rouleau de guidage de courroie (3) du deuxième transporteur à courroie (B) sont fabriqués à partir d'un non-métal et, de plus, le rouleau de guidage de courroie (3) est spécifié comme étant un rouleau non entraîné.

5. Procédé de séparation magnétique comprenant les étapes consistant à :
utiliser le séparateur magnétique selon l'une quelconque des revendications précédentes, et
fournir un matériau pulvérulent et granulaire (a) d'un dispositif d'alimentation (6) au premier transporteur à courroie (A) avec une épaisseur de couche supérieure au diamètre de la plus petite particule contenue dans le matériau pulvérulent et granulaire (a), et dans lequel
la fréquence de changement de champ magnétique F en Hz, qui est définie par la formule (1) suivante, du rouleau magnétique (4r) est spécifiée comme étant supérieure ou égale à 170 Hz, $F = \left(x⋅P\right) / 60$ où x : le nombre de tours par minute du rouleau magnétique(4r)
P : le nombre de pôles magnétiques (5) fournis au rouleau magnétique (4r), dans lequel une paire du pôle nord et du pôle sud est comptée comme un pôle magnétique.

6. Procédé de séparation magnétique selon la revendication 5, dans lequel la courroie transporteuse (1) du premier transporteur à courroie (A) et la courroie transporteuse (2) du deuxième transporteur à courroie (B) sont déplacées dans les mêmes directions ou dans les directions inverses l'une de l'autre dans la partie de bord de fin de transporteur (10) du premier transporteur à courroie (A) et la partie de bord de début de transporteur (11) du deuxième transporteur à courroie (B).

7. Procédé de fabrication d'une source de fer pour produire la source de fer à partir d'un sous-produit d'un processus de fabrication de fer, comprenant l'étape d'utilisation du séparateur magnétique selon l'une des revendications 1 à 4 ou le procédé de séparation magnétique selon la revendication 5 ou 6.
